

## UNITED STATES PATENT OFFICE

2,135,426

## TREATMENT OF STILL RESIDUE

Frank W. Corkery, Clairton, Pa., assignor to  
Pennsylvania Industrial Chemical Corporation,  
a corporation of Pennsylvania

No Drawing. Application July 2, 1936, Serial  
No. 88,591. Renewed March 19, 1938

4 Claims. (Cl. 106—31)

This invention relates to the treatment of still residue by oxidation, and more particularly to the treatment of the still residue in preparation for oxidation.

5 The still residue with which I deal is a still residue remaining from the treatment of coke-oven light oil. This still residue contains polymers of resin-forming bodies in various stages of polymerization, heavy monomers, naphthalene, and varying percentages of solvents and sulphonates. It is a dark, viscous, oily substance deficient in drying qualities, and of itself possessing but little utility in the arts. In my co-pending applications Serial No. 53,213, filed 10 December 6, 1935, Serial No. 54,852, filed December 17, 1935, and Serial No. 62,045, filed February 3, 1936, I have respectively disclosed methods of producing useful products by oxidizing the total content of still residue by itself to form 15 an elastic body, of oxidizing the still residue in association with a non-mineral pitch, and of oxidizing the still residue in association with a drying oil.

It should be understood that still residue as 20 commercially available is not uniform in its content and qualities. The light oil from which the still residue has its immediate derivation is chiefly obtained from the gases coming off during the by-product coking of coal. As this operation is performed usually at plants directly 25 associated with large steel companies, and as these companies follow variant procedure in treating and fractionating the by-product yield, still residue from some sources cannot be treated 30 identically with that from other sources. Thus many still residues have a content of sulphonates so low that no treatment for their removal is necessary. Other still residues contain sulphonates in such proportions that it is of importance to remove them prior to oxidizing the 35 still residue. It is with still residue of this latter type that the initial stages of my preparatory treatment are concerned.

In preparation of still residues containing a 40 large content of sulphonates and/or sulphates resultant from the purification of the light oil and light oil fractions, to obtain from them a clear oxidized product free from objectionable odor, I make specific adaptation of the solvent 45 separation principle. In so doing, I commingle the still residue with a suitable petroleum distillate, such as petroleum naphtha, mineral spirits, kerosene, ligroin, gasoline, and the like, in which the sulphonates and sulphates are relatively insoluble. Upon commingling the petroleum dis-

tillate with the still residue, without heating, there occurs a precipitation of the sulphonates and sulphates from the solution. I have found that any substantial quantity of the petroleum distillate causes precipitation of sulphonates and sulphates, but have also found that, if the initial content of sulphonates or sulphates is substantial, adequate removal of them is not effected unless the volume of petroleum distillate is at least equal to the volume of the still residue. 5

To describe my preferred conditions, I have found that within the ratio of from 2 to 5 volumes of petroleum distillate to each volume of still residue precipitation of sulphonates and/or sulphates present in any quantity in the still residue is substantially complete. If the petroleum distillate approaches in quantity 5 volumes of the petroleum distillate to each volume of the still residue, the conditions being otherwise suitable, separation of the precipitate from the solution may be effected merely by permitting the suspension to settle. By commingling the still residue with petroleum distillate to form a solution therewith at normal room temperature, the precipitate is of a granular, readily separable 10 nature. At substantially higher temperatures the precipitate does not form in this granular condition. It is desirable, therefore, in cases where the solution is made under extraordinarily high atmospheric conditions, and cases in which the still residue has become spontaneously heated, to cool the solution to a temperature not exceeding 80° F. 15

The precipitate comprises the sulphonates and sulphates initially present in the still residue, 20 and may have associated with them traces of other foreign matter insoluble in the petroleum distillate. If a mere settling is inadequate to effect separation of the precipitate from the solution of still residue in the petroleum distillate, 25 separation of the solution and precipitate is effected by filtration. After separation of the precipitate, the still residue solution is agitated with a small quantity of sodium hypochlorite followed by a sodium hydroxide wash, and water 30 washing. These agents cooperate in rendering removable from the solution impurities which are soluble in the petroleum distillate; thus purifying the solution generally, and eliminating the disagreeable sweetish odor which is a characteristic of untreated still residue. 35

I then introduce into the solution bleaching clay of any of the well known sorts, desirably in a weight of from 2 to 5 per cent. the weight of the solution, agitate it in the solution, and filter it 40

out. The clay, as filtered from the solution, carries with it some of the color-forming bodies of the still residue; leaving the solution improved in color as well as odor, and containing a lessened content of impurities.

Following the clay treatment, the still residue is recovered from solution by distilling over the petroleum distillate in which it is dissolved. This distillation desirably is carried to a temperature of approximately 425° F. under vacuum, in order wholly to remove naphthalene and the solvent content of the still residue. It is possible to utilize straight distillation up to a temperature of from 390° F. to 400° F., distilling under vacuum only in the high temperature range.

Still residue so treated is in good condition for oxidation into the form of a residual gum by blowing air or undiluted oxygen therethrough, or for a similar oxidizing treatment in admixture with a drying oil such as linseed oil, fish oil, or the like. It may also be oxidized as it is in admixture with a non-mineral pitch, such as cottonseed pitch, stearin pitch, and the like. I have discovered, however, that compatibility of the still residue and the pitch as oxidized together may be brought closer to the absolute, and the qualities of the product may otherwise be improved by removing a portion of such oily content of the purified still residue as is not formed of the higher polymer content of the still residue. This is for the reason that non-mineral pitch possesses itself, when oxidized, considerable elasticity; and also for the reason that (unlike the drying oils) a degree of incompatibility between the still residue and the pitch develops when a high stage of oxidation has been reached in a mixture of still residue and pitch.

Taking then a topped still residue freed of sulphonates and other impurities, and stripped of a portion of its lower boiling end, it is commingled with a pitch of non-mineral origin in a vessel equipped with heating means and with means for forcing gases therethrough. As a desirable procedure, the temperature of the pitch is raised in the treating vessel to the melting-point of the pitch before the still residue is introduced and mixed with the pitch, but in any event the temperature of the mixture is raised to at least the melting-point of the pitch before blowing is begun.

During a relatively extended blowing period, heat is supplied to the vessel adequate to maintain the mixture at such temperature that it is in condition suitable for the dispersion of oxygen therethrough. As oxidation proceeds, it is necessary progressively to increase the temperature of the mixture in order that it may sufficiently be liquid for the oxygen dispersion. I have found a temperature progressively raised within the range of 160° F. to 300° F. suitable for the oxidizing treatment. When, as is most convenient, air is the source of oxygen, blowing desirably is continued for from 3 to 5 days. When pure, or relatively pure, oxygen is used an appropriately shortened treating period suffices to bring the mixture to an equal stage of oxidation.

The resultant product is an elastic mass, which is clear and of light color, and which is soluble in the aromatic hydrocarbon solvents. Depending upon the proportion of pitch to still residue, and the stage to which oxidation is carried, it is soluble in the varying percentage mixtures of aromatic solvents. I have found a composite of equal volumes of still residue and non-mineral

pitch brought to a stage of oxidation at which the composite melts at a temperature of about 160° F. to be a product of great utility. For example, it is highly useful as a component of mastic tile, being compatible with ester gum, 5 coumarone resin, and other materials commonly used as tile components. It is capable of taking delicate tints, and is highly elastic. In this connection it may be noted that I deliberately leave in the still residue some portion of its 10 lighter oily content, in order that adequate elasticity of the product may be obtained. The composite product is also useful for the waterproofing of paper, fabric, and other normally absorbent materials.

The relative proportions of the still residue and the non-mineral pitch in the composite may be varied within relatively wide limits from equality one with the other without substantial loss in any of the qualities of elasticity and solubility of the product, and without impairing the compatibility of the components of the composite. It may be noted that the composite product remains clear and bright throughout a pulling test, thus indicating substantially complete removal of sulphonates.

In preparation for mixture and blowing, I desirably remove 25% to 75% of the lighter oil end of the still residue as it exists after purification, and after the removal of solvents and 20 naphthalene. The extent to which the still residue is advantageously stripped depends upon the proportional quantity of the still residue included in the composite, and the stage of oxidation to which it is carried. The elasticity of 25 the product, or, as otherwise expressed, the penetration of the product, depends upon the content of the oily lower polymers remaining in the still residue. In no event, however, do I find it desirable wholly to deprive the still residue of its 40 content of lower polymers.

When the preparation of a still residue of the specified type (a still residue from the treatment of coke-oven light oil) involves a purification such as that outlined above, the removal 45 of a portion of the lower polymer oils may follow as an incident to distilling off the mineral spirits used in purification and the initial solvent and naphthalene content of the still residue. In such case distillation under vacuum at 50 50 a temperature at and above 425° F. is continued until the still residue has been stripped of the desired quantity of its oily, lower boiling end.

In preparing a still residue which need not be subjected to the preliminary purification, it may 55 none the less be stripped of a portion of its oily, lower boiling content in similar manner, as a step preparatory to its oxidation. While it has been stated above that purification need not be practiced upon some still residues, it may be desirable to remove sulphonates even from still residues containing a relatively small proportion of them when a product of particular purity is desired.

The removal of a portion of the lower boiling, 65 oily constituents of the still residue is, as stated above, generally desirable only in preparation of the still residue for oxidation in association with pitch to give a pitchy composite. In rare instances, it may be practiced to modify the 70 procedure in producing a residual gum disclosed in my co-pending application Serial No. 53,213, reference to which has been made above. It is appropriate when for some purpose a product of decreased elasticity and penetration may be 75

- desired. In such event the still residue, deprived of a portion of its oily, lower boiling content, is subjected by itself to oxidation. The method of oxidization is similar to blowing air or oxygen 5 in less dilute condition through the stripped still residue while supplying to the still residue heat adequate to maintain it in condition suitable for the oxygen dispersion. As compared with the procedure disclosed in detail in my application 10 Serial No. 53,213, the period of treatment may be shortened because of the reduced lower boiling content of the still residue, 3 or 4 days of blowing treatment with air being adequate for the production of a gum which is solid at temperatures 15 higher than normal room temperature. The removal of a portion of the oily, lower boiling content prior to oxidation may be practiced on the still residue whether or not it has been subjected to a purifying treatment.
- 20 It may be explained that the absence of sulphonates in a product such as the oxidized composite pitch, oxidized composite of still residue and drying oil, or oxidized still residue alone substantially improves the solubility of the resultant 25 product, and also to some extent improves its waterproofing qualities.

In connection specifically with the oxidized composite of still residue and non-mineral pitch, the removal of a portion of the oily lower polymers of the still residue serves substantially to improve the compatibility of the components and the solubility of the composite when carried to a relatively high stage of oxidation at which it acquires a melting-point of 150° F. and higher. 30 In the modified pitch this advantage accompanies the advantage of avoiding an elasticity so high as to be undesirable for certain uses, such as its use in tile manufacture.

I claim as my invention:

- 40 1. The herein described method of oxidizing liquid aromatic still residue from the treatment of coke-oven light oil initially containing sulphonates and like impurities in association with non-mineral pitch to produce an oxidized pitchy composite of light color and transparent in a film the components of which are in a condition of approximately absolute compatibility, which comprises precipitating the sulphonates and like impurities of the still residue by solvent separation in a petroleum distillate, separating out the precipitate, by distillation separating from the still residue the petroleum distillate and the lower boiling end of the still residue including a portion of the oily lower polymers thereof; and 45 oxidizing in admixture the still residue so purified and prepared with a pitch of non-mineral origin

by oxygen dispersion through a mixture of the still residue and pitch while supplying to the mixture heat adequate to maintain it at a progressively increased liquefying temperature.

2. The herein described method of oxidizing 5 liquid aromatic still residue from the treatment of coke-oven light oil in association with non-mineral pitch to produce an oxidized pitchy composite of light color and transparent in a film the components of which are in a condition of 10 approximately absolute compatibility, which comprises removing a portion and less than all of the oily lower polymers of the still residue; and oxidizing in admixture the still residue so prepared and pitch of non-mineral origin by 15 oxygen dispersion through a mixture of the still residue and pitch while supplying to the mixture heat adequate to maintain it at a progressively increased liquefying temperature.

3. The herein described method of oxidizing 20 liquid aromatic still residue from the treatment of coke-oven light oil initially containing sulphonates and like impurities in association with non-mineral pitch to produce an oxidized pitchy composite of light color and transparent in a film, 25 the components of which are in a condition of approximately absolute compatibility, which comprises freeing the raw still residue of sulphonates and like impurities, removing from the still residue which has been freed of sulphonates a portion of the lower oily polymers thereof, and oxidizing in admixture the still residue so purified and prepared with a pitch of non-mineral origin by 30 oxygen dispersion through a mixture of still residue and pitch while supplying to the mixture 35 heat adequate to maintain it at a progressively increased liquefying temperature.

4. The herein described method of oxidizing liquid aromatic still residue from the treatment of coke-oven light oil initially containing sulphonates and like impurities in association with non-mineral pitch to produce an oxidized pitchy composite of light color and transparent in a film, the components of which are in a condition of approximately absolute compatibility, 45 which comprises removing the sulphonates and like impurities from the raw still residue, and oxidizing in admixture the still residue purified by removal of sulphonates and pitch of non-mineral origin by oxygen dispersion through a 50 mixture of the still residue and pitch while supplying to the mixture heat adequate to maintain it at a progressively increased liquefying temperature.

FRANK W. CORKERY. 55